

## UNITED STATES PATENT OFFICE

2,138,950

## METHOD OF PRODUCING YARN

William Whitehead, Cumberland, Md., assignor  
to Celanese Corporation of America, a corpora-  
tion of Delaware

No Drawing. Application March 16, 1937,  
Serial No. 131,185

2 Claims. (Cl. 117—21)

This invention relates to the manufacture of 5  
yarns and fabrics and especially to plied yarns  
containing ends of high twist of both directions  
and ends of low twist of both directions, which  
plied yarns will handle without difficulty on weaving  
and knitting devices.

An object of the invention is the economic and 10  
expeditious production of plied yarns having a  
high weaving and knitting efficiency. Another  
object of the invention is the production of a plied  
yarn having ends of both right and left hand  
twist which is so balanced that the ends having  
one twist do not snap, or break, before the ends  
of the opposite twist when the yarn is under ten- 15  
sion. Other objects of the invention will appear  
from the following detailed description.

The plying of a plurality of ends of yarn to 20  
form a plied or doubled yarn has been practiced  
for some time, for the most part for the purpose  
of producing a uniform yarn under the theory  
that the weak or thin places in the various ends  
would not likely fall together in the plied yarn. 25  
This evenning up of the yarn is unnecessary with  
yarns formed of substantially continuous artificial  
filaments as each yarn is substantially uniform  
in denier. However, by plying 2, 3, 4 or  
more ends of such yarn, different types of yarn 30  
and, therefore, different types of fabric may be  
produced. Plied yarn at least one end of which  
has a high degree of twist, say, 20 or more turns  
per inch, has heretofore been defective in several  
respects. Ordinarily, plied yarn made from con- 35  
tinuous filaments tends to curl or spiral upon it-  
self in weaving and knitting operations and, also,  
when the yarn is placed under a stress the end  
having a high degree of twist tends to snap first.  
In effect, the plied yarn containing at least one 40  
end having a high degree of twist, as heretofore  
commonly manufactured, is not as strong as the  
total strength of the ends, as the end having a  
high degree of twist snaps first, leaving the other  
end or ends to bear the load. Furthermore, upon 45  
the breaking of the end having a high degree of  
twist, the broken ends fly out of the yarn and  
catch on needles, heddles, etc. Even if the yarn  
is not completely broken and the ends do not  
catch in the eyes of the weaving or knitting de- 50  
vices, the loss of tension on the end having the  
high degree of twist produces a defect in the fab-  
ric formed from the yarn.

I have now found that if the plied yarn is built  
up in such a manner that the twists in the vari-  
ous components are balanced in the yarn as the  
yarn lies in the fabric, a much stronger yarn is  
produced. This type of yarn does not curl or 5  
spiral upon itself in weaving and knitting opera-  
tions and, as the strength of the yarn is nearly  
that of the combined total strength of all the  
ends, it knits with much better efficiency than the  
plied yarns as heretofore made. 10

In accordance with my invention, I form a yarn  
by twisting together a plurality of ends of yarn in  
such a manner that there is in the various com-  
ponents of the yarn, as said yarn lies in a fabric,  
a balanced amount of twist. This invention, I 15  
find, is of particular importance in forming yarns  
from a plurality of ends at least one end of which  
has a high degree of twist and consists of sub-  
stantially continuous artificial filaments.

Although this invention is applicable to the for- 20  
mation of yarns from any suitable fiber or fila-  
ment, or both, it is particularly applicable to the  
formation of yarns containing fibers or filaments  
of an organic derivative of cellulose such as the  
organic esters of cellulose and cellulose ethers. 25  
Examples of organic esters of cellulose are cel-  
lulose acetate, cellulose propionate, cellulose for-  
mate and cellulose butyrate, while examples of  
the cellulose ethers are ethyl cellulose, methyl  
cellulose and benzyl cellulose. 30

Yarns of other materials may be employed in  
building the yarn in accordance with this inven-  
tion. The other yarns may be employed alone or  
with yarns containing organic derivatives of cel-  
lulose. Examples of other filaments or fibers 35  
which may be employed to form the yarns are  
regenerated or reconstituted cellulose made by  
either the cuprammonium or viscose methods,  
silk, cotton, wool, etc. The fibers and filaments  
of organic derivatives of cellulose may be em- 40  
ployed alone in forming a single end, or fibers or  
filaments of an organic derivative of cellulose  
may be mixed with other fibers or filaments to  
form a single end or ends, each of which con-  
tains a single type of fiber or filament. 45

When artificial fibers or filaments such as  
those containing organic derivatives of cellulose  
or reconstituted or regenerated cellulose are em-  
ployed, these may have effect materials placed  
therein during their formation. These effect 50

materials may be dyes, lakes, pigments, fillers, plasticizers, fire retardants, etc.

A balanced amount of twist in the plied yarn means that in the said yarn the ends make up substantially equally sized cross sections of yarn of opposite and substantially equal twist. For instance, two 40 denier ends having 45 turns per inch left hand twist may be plied with 5 turns per inch left hand twist with one end of 80 denier 10 having 55 turns per inch right hand twist. As this yarn lies in a fabric there will be 80 denier of yarn having 50 turns per inch right hand twist and 80 denier of yarn having 50 turns per inch left hand twist. An absolute balance is not necessary but it is preferred within the limits of 15 modern machinery and large scale production methods. A yarn is balanced, insofar as this invention is concerned, when the right hand twist is within 8% of the left hand twist. This limit 20 also holds for the overall denier of the end or ends of the right hand twisted sections as compared with the left hand twisted sections.

The invention is applicable to the plying of ends of yarn each end of which may have any 25 degree of twist from 0 to 100 or more turns per inch, and each end may be of any suitable denier or count so long as there is a balancing component in the plied yarn. This invention is particularly applicable to the production of a four 30 component yarn made entirely of continuous filaments containing an organic derivative of cellulose, which yarn has ends of crepe twisted or tightly twisted yarn and ends of normal twist or small amount of twist. For instance, the invention is applicable to the production of yarns 35 containing four ends, one end of right hand twist and one end of left hand twist having more than 20 turns per inch, say, between 60 and 90 turns per inch, while the other ends have less than 20 turns per inch.

As an illustration and not as a limitation, the following example is given. All the ends in the following example are 100 denier and all are formed from continuous filaments of cellulose acetate.

#### Example

A two end plied yarn is formed from one end having 65 turns per inch right hand twist doubled with 6 turns per inch of right hand twist with an 50 end having 5 turns per inch right hand twist. Another two end plied yarn is formed from one end having 65 turns per inch left hand twist doubled 16 turns per inch left hand twist with one end of yarn having 5 turns per inch left hand 55 twist. These two plied yarns are then plied with 5 turns per inch right hand twist. This produces a yarn having a balanced twist, as said yarn lies in the fabric. To aid in visualizing this example the following graphs are given wherein S means 60 right hand twist and Z means left hand twist:



As the yarn lies in the fabric, the twist is then:



The yarns may be steamed on the bobbin, spool, quill, etc., before, between and/or after each plying operation. The yarn may also be steamed during the actual insertion of the twist in the same. The steaming of the yarns is of especial importance when the yarns contain a thermoplastic derivative of cellulose and there is inserted into the yarn a twist of more than 20 turns per inch. The steaming of the yarns may be accomplished by leading the yarns through a steam chamber mounted on the twisting or plying device. In place of steam other methods of heating the thermoplastic yarn may be employed, such as contacting the yarn with a heated roller or other element.

Obviously, the adding or subtracting twist in plying operations influences the length of the ends and, therefore, indirectly the amount of twist per unit length.

It is understood that the foregoing detailed description is given merely by way of illustration and that many variations may be made therein without departing from the spirit of my invention.

Having described my invention, what I desire to secure by Letters Patent is:

1. In a method of producing a balanced yarn by plying four ends of yarn together, the steps of twisting separately two ends in opposite directions equally and to more than 20 turns per inch, twisting separately two ends in opposite directions equally and to less than 20 turns per inch, plying the two ends of the same direction (direction A) with a direction A twist, plying the two ends of the opposite direction (direction B) with a direction B twist equal to the plying twist inserted in plying the direction A twisted end plus two times the amount of twist to be inserted in plying the two plied ends and plying the two plied ends with a direction A twist.

2. In a method of producing a balanced yarn by plying four ends of yarn together, the steps of twisting separately two ends in opposite directions equally and to more than 20 turns per inch, twisting separately two ends in opposite directions equally and to less than 20 turns per inch, steaming the yarns, plying the two ends of the same direction (direction A) with a direction A twist, plying the two ends of the opposite direction (direction B) with a direction B twist equal to the plying twist inserted in plying the direction A twisted end plus two times the amount of twist to be inserted in plying the two plied ends, plying the two plied ends with a direction A twist and steaming the yarns.